



US009695378B2

(12) **United States Patent**  
**Hayama et al.**

(10) **Patent No.:** **US 9,695,378 B2**  
(b5) **Date of Patent:** **Jul. 4, 2017**

- (54) **SLIDING MECHANISM AND GREASE COMPOSITION FOR SLIDING MECHANISMS**
- (71) Applicant: **NISSAN MOTOR CO., LTD.**, Yokohama-shi, Kanagawa (JP)
- (72) Inventors: **Makoto Hayama**, Chigasaki (JP); **Terasu Yoshinari**, Chigasaki (JP); **Masanori Komaba**, Sendai (JP); **Yutaka Mabuchi**, Yokohama (JP); **Yoshiteru Yasuda**, Yokohama (JP); **Saburo Abe**, Ebina (JP); **Katsuyuki Serizawa**, Isehara (JP); **Tsuyoshi Higuchi**, Yokohama (JP)
- (73) Assignee: **NISSAN MOTOR CO., LTD.**, Yokohama-shi (JP)
- (\*) Notice: Subject to any disclaimer, the term of this patent is extended or adjusted under 35 U.S.C. 154(b) by 0 days.

- (21) Appl. No.: **14/389,901**
- (22) PCT Filed: **Mar. 29, 2013**
- (86) PCT No.: **PCT/JP2013/059552**  
§ 371 (c)(1),  
(2) Date: **Oct. 1, 2014**
- (87) PCT Pub. No.: **WO2013/150975**  
PCT Pub. Date: **Oct. 10, 2013**

- (65) **Prior Publication Data**  
US 2015/0072906 A1 Mar. 12, 2015
- (30) **Foreign Application Priority Data**  
Apr. 2, 2012 (JP) ..... 2012-084108

- (51) **Int. Cl.**  
**C10M 171/02** (2006.01)  
**C10M 169/04** (2006.01)  
**C10M 117/02** (2006.01)  
**F16C 31/04** (2006.01)  
**C10N 40/02** (2006.01)  
**C10M 169/02** (2006.01)
- (52) **U.S. Cl.**  
CPC .. **C10M 169/02** (2013.01); **C10M 2203/1006** (2013.01); **C10M 2205/0285** (2013.01); **C10M 2207/0406** (2013.01); **C10M 2207/1285** (2013.01); **C10M 2207/2825** (2013.01); **C10M 2209/1033** (2013.01); **C10N 2220/022** (2013.01); **C10N 2230/06** (2013.01); **C10N 2240/02** (2013.01); **C10N 2250/10** (2013.01); **C10N 2280/00** (2013.01)

- (58) **Field of Classification Search**  
CPC ..... C10M 2207/1285; C10M 2210/01; C10M 169/02; C10M 2205/0285; C10M 2207/2825; C10M 2209/1033; C10M 2203/1006; C10M 2207/0406; C10N 2280/00; C10N 2250/10; C10N 2240/02; C10N 2220/022; C10N 2230/06; C10N 2210/01

See application file for complete search history.

- (56) **References Cited**
- U.S. PATENT DOCUMENTS
- |                   |         |                      |         |
|-------------------|---------|----------------------|---------|
| 4,859,352 A *     | 8/1989  | Waynick .....        | 508/174 |
| 5,714,444 A       | 2/1998  | Yokouchi et al.      |         |
| 7,228,786 B2 *    | 6/2007  | Hamada et al. .....  | 92/155  |
| 7,771,821 B2      | 8/2010  | Martin et al.        |         |
| 8,445,415 B2      | 5/2013  | Mabuchi et al.       |         |
| 2005/0064196 A1   | 3/2005  | Martin et al.        |         |
| 2007/0292711 A1 * | 12/2007 | Ueno et al. .....    | 428/688 |
| 2008/0194441 A1 * | 8/2008  | Kawata et al. .....  | 508/208 |
| 2011/0034357 A1 * | 2/2011  | Kawata et al. .....  | 508/202 |
| 2011/0136708 A1 * | 6/2011  | Mabuchi et al. ..... | 508/122 |

## FOREIGN PATENT DOCUMENTS

- |    |                    |         |
|----|--------------------|---------|
| CN | 1833018 A          | 9/2006  |
| EP | 1479946 A2 *       | 11/2004 |
| EP | 1510594 A2         | 3/2005  |
| EP | 2316912 A1         | 5/2011  |
| JP | 8-143884 A         | 6/1996  |
| JP | 2002-363590 A      | 12/2002 |
| JP | 2003-181185 A      | 7/2003  |
| JP | 2006-194281 A      | 7/2006  |
| JP | 2010-053236 A1     | 3/2010  |
| WO | WO 2006075219 A2 * | 7/2006  |
| WO | WO 2010/001784 A1  | 1/2010  |
| WO | WO 2010001784 A1 * | 1/2010  |

## OTHER PUBLICATIONS

- Emery Synthetic Lubricant Basestocks Technical Data Sheet #2033A-7/2000.\*  
Extended Search Report issued in European Patent Application No. 13772304.5 dated Mar. 10, 2015.

\* cited by examiner

Primary Examiner — Pamela H Weiss

(74) Attorney, Agent, or Firm — Foley &amp; Lardner LLP

(57) **ABSTRACT**

A sliding mechanism includes first and second members slidably relative to each other and a grease composition interposed between the first and second members and containing a thickening agent and a base oil, wherein the grease composition contains lithium 12-hydroxystearate as the thickening agent and dioctyl sebacate and/or poly- $\alpha$ -olefin as the base oil; and wherein at least one of the first and second member has a sliding surface coated with a hard carbon film of diamond-like carbon.

**5 Claims, No Drawings**

## 1

**SLIDING MECHANISM AND GREASE  
COMPOSITION FOR SLIDING  
MECHANISMS**

**FIELD OF THE INVENTION**

The present invention relates to a sliding mechanism. More particularly, the present invention relates to a sliding mechanism in which sliding members are slideable via a hard carbon film in the presence of a specific grease and a grease composition therefor.

**BACKGROUND ART**

In automotive vehicles, sliding materials play a role in imparting high wear resistance and low friction coefficients to engine sliding parts under extreme friction/wear conditions. It has recently been attempted to apply various hard thin film materials and roller rocker arms with roller needle bearings to follower parts such as valve lifters and lifter shims.

Hard carbon materials, in particular diamond-like carbon (DLC) materials, are expected as low-friction sliding materials due to the fact that the hard carbon materials generally show low friction coefficients in the air in the absence of lubricating oils than those of wear-resistant hard coating materials such as titanium nitride (TiN) and chromium nitride (CrN).

Further, Patent Document 1 discloses a sliding mechanism that attains low-friction characteristics by the use of sliding members, at least one of which has a hard carbon coating formed of DLC with a hydrogen content of 20 atomic % or less, in combination with a grease containing an ester oil, an ether oil or a mixture thereof as a base oil.

There has however been a demand to achieve further friction reduction in terms of resource conservation and energy conservation. It is accordingly an object of the present invention to provide a sliding mechanism capable of showing a lower friction coefficient for friction reduction and, at the same time, improving in wear resistance and a grease composition for use in such a sliding mechanism.

**PRIOR ART DOCUMENTS**

Patent Document

Patent Document 1: Japanese Laid-Open Patent Publication No. 2006-194281

**SUMMARY OF THE INVENTION**

As a result of extensive research, the present inventors have newly found that the use of lithium 12-hydroxystearate (Li—(12OH)St) as a thickening agent makes it possible that not only ester and ether oils but also poly- $\alpha$ -olefin can effectively act to reduce frictions between sliding members in sliding mechanisms. The present inventors have also found that dioctyl sebacate, which is one kind of dibasic acid ester, has a particularly good friction reducing effect as compared to other ester oils. Namely, the present invention includes the following aspects.

## 2

1. A sliding mechanism, comprising:  
first and second members slideable relative to each other;  
and  
a grease composition interposed between the first and second members and containing a thickening agent and a base oil,  
wherein the grease composition contains lithium 12-hydroxystearate as the thickening agent and dioctyl sebacate and/or poly- $\alpha$ -olefin as the base oil; and  
wherein at least one of the first and second member has a sliding surface coated with a hard carbon film of diamond-like carbon.
2. The sliding mechanism according to the above aspect 1,  
wherein the base oil has a kinematic viscosity of 10 to 70 mm<sup>2</sup>/sec at 40° C.
3. The sliding mechanism according to the above aspect 1 or 2,  
wherein the hard carbon film of diamond-like carbon has a hydrogen content of 0.5 atomic % or less.
4. A grease composition for a sliding mechanism, the sliding mechanism comprising first and second members slideable relative to each other with the grease composition interposed therebetween, at least one of the first and second members having a sliding surface coated with a hard carbon film of diamond-like carbon, the grease composition comprising:  
a thickening agent; and  
a base oil,  
wherein the grease composition contains lithium 12-hydroxystearate as the thickening agent and dioctyl sebacate and/or poly- $\alpha$ -olefin as the base oil.
5. The grease composition for the sliding mechanism according to the above aspect 4, wherein the base oil has a kinematic viscosity of 10 to 70 mm<sup>2</sup>/sec at 40° C.  
It is possible that the sliding mechanism and the grease composition therefor according to the present invention can achieve further friction reduction. It is also possible that the sliding mechanism and the grease composition therefor according to the present invention can achieve high wear resistance.

**DESCRIPTION OF EMBODIMENTS**

[Grease Composition]  
(Thickening Agent)

The grease composition of the present invention contains Li—(12OH)St as a thickening agent. In the present invention, any other thickening agent may be contained within the range that does not impair the performance of the grease composition. Examples of the other thickening agent are:  
metal soap thickening agents such as metal soaps of Li, Na etc. and composite metal soaps of any combination selected from Li, Na, Ba, Ca etc.; and non-soap thickening agents such as Benton, silica gels and urea compounds. The urea compounds can be diurea compounds, triurea compounds, tetraurea compounds, polyurea compounds, urea-urethane compounds, diurethane compounds and mixtures thereof. It is however most preferable to use Li—(12OH)St solely as the thickening agent.

The amount of the thickening agent contained in the composition is preferably 2 to 40 mass %, more preferably 5 to 30 mass %, still more preferably 8 to 25 mass %. In the

case of using the other thickening agent, the amount of Li—(12OH)St contained in the thickening agent is preferably 50 to 100 mass %, more preferably 70 to 100 mass %, based on the total mass of the thickening agent.

(Base Oil)

The grease composition of the present invention contains dioctyl sebacate, which is one kind of dibasic acid ester, and/or poly- $\alpha$ -olefin as a base oil. The use of such a base oil leads to reduction of friction coefficient and improvement of wear resistance.

If the kinetic viscosity of the base oil is too low, it is not possible to obtain adequate wear resistance due to oil film breakage. If the kinetic viscosity of the base oil is too high, it is difficult to feed the grease composition to the lubrication part due to flowability deterioration. For these reasons, the kinetic viscosity of the base oil is preferably 10 to 70 mm<sup>2</sup>/s, more preferably 10 to 50 mm<sup>2</sup>/s, at 40° C.

(Additives)

The grease composition of the present invention may contain, as additives, a rust inhibitor, a load-carrying additive, an antioxidant and the like as needed. The amount of these additives contained is generally 0.01 to 10 mass %.

The rust inhibitor can be either an inorganic rust inhibitor or an organic rust inhibitor. Examples of the inorganic rust inhibitor are inorganic metal salts such as sodium silicate, sodium nitrite, sodium molybdate, lithium carbonate and potassium carbonate. Examples of the organic rust inhibitor are: benzoates such as sodium benzoate lithium benzoate; sulfonates such as calcium sulfonate and zinc sulfonate; carboxylates such as zinc naphthenate and sodium sebacate; succinic acid; succinic acid derivatives such as succinic anhydride and succinic acid half ester; sorbitan esters such as sorbitan monooleate and sorbitan trioleate; and fatty acid amine salts.

The load-carrying additive can be a phosphorus-based load-carrying additive such as phosphoric ester, a sulfur-based load-carrying additive such as polysulfide or sulfurized grease, a phosphorus-sulfur-based load-carrying additive such as phosphorothioate, or other load-carrying additive such as thiocarbamate, thiophosphate or organophosphate. There can also be used a solid lubricant such as MoS<sub>2</sub>, graphite, MCA (melamine cyanurate), PTFE (polytetrafluoroethylene) or the like as the load-carrying additive.

The antioxidant is known for prevention of grease oxidation degradation and can be a phenol-based antioxidant or an amine-based antioxidant. Examples of the phenol-based antioxidant are 2,6-di-tertiary-butyl-p-cresol (BHT), 2,2'-methylenebis(4-methyl-6-tertiary-butylphenol), 4,4'-butanlylidynabis(3-methyl-6-tertiary-butylphenol), 2,6-di-tertiary-butylphenol, 2,4-dimethyl-6-tertiary-butylphenol, tertiary-butylhydroxyanisole (BHA), 4,4'-butanlylidynabis(3-methyl-6-tertiary-butylphenol), 4,4'-methylenebis(2,3-di-tertiary-butylphenol) and 4,4'-thiobis(3-methyl-6-tertiary-butylphenol). Examples of the amine-based antioxidant are N-n-butyl-p-aminophenol, 4,4'-tetramethyl-di-aminodiphenylmethane,  $\alpha$ -naphthylamine, N-phenyl- $\alpha$ -naphthylamine and phenothiazine.

[Sliding Mechanism]

(Diamond-like Carbon)

The sliding mechanism of the present invention has first and second sliding members slidable relative to each other in the presence of the grease composition. At least one of

these sliding members has a sliding portion coated with a hard carbon film of diamond-like carbon (DLC).

Herein, the hard carbon film refers to a thin film of amorphous carbon-containing DLC in which carbon atoms are bonded by both of diamond bond (sp<sup>3</sup> bond) and graphite bond (sp<sup>2</sup> bond).

Specific examples of the DLC are: a-C (amorphous carbon) consisting only of carbon; a-C:H (hydrogen amorphous carbon) containing hydrogen; and MeC containing in a part thereof as a metal atom such as titanium (Ti) or molybdenum (M). It is preferable in the present invention that the hydrogen content of the DLC is low. Preferably, the hard carbon film is formed of DLC with a hydrogen content of 0.5 atomic % or less. It is more preferable that the hard carbon film is formed of hydrogen-free a-C type (amorphous carbon type) DLC.

(Base Material)

There is no particular limitation on the base materials of the first and second sliding members in the sliding mechanism of the present invention. There can preferably be used iron-based alloy such as steel as the base material of the sliding member.

In the present invention, the sliding mechanism allows sliding between the sliding members with the grease composition being interposed between the sliding surface of one of the sliding members and the DLC hard carbon film on the sliding surface of the other of the sliding members or sliding between the sliding members with the grease composition being interposed between the DLC hard carbon films on the respective sliding surfaces of the sliding members. In such sliding, there is no particular limitation on the friction/sliding form. The sliding can be allowed in any of point contact form, line contact form or surface contact form in the sliding mechanism of the present invention.

It is feasible to apply the sliding mechanism of the present invention to various sliding mechanisms where grease lubrication is required under the conditions of relatively high temperature and high pressure. The sliding mechanism can suitably be applied to sliding mechanism for automotive vehicles although there is no particular limitation on the type of the machine or apparatus to which the sliding mechanism is applied.

As described above, it is possible according to the present invention to achieve reduction of friction coefficient and improvement of wear resistance by the use of the sliding members, at least one of which has its sliding portion coated with DLC, in combination with the grease composition containing Li—(12OH)St as the thickening agent and dioctyl sebacate and/or poly- $\alpha$ -olefin as the base oil. Although the present invention is not limited to any theory, it is considered that Li—(12OH)St acts favorably on the DLC film in the boundary lubrication and mixed lubrication regions so as to provide a low friction coefficient in the present invention. This effect becomes small when the kinetic viscosity of the base oil becomes high so that the oil film increases in thickness to cause relatively less participation of Li—(12OH)St in lubrication. Thus, the kinetic viscosity of the base oil is preferably 10 to 70 mm<sup>2</sup>/sec at 40° C. in order to secure good lubrication. The reason for showing good friction/wear performance by the combined use of the poly- $\alpha$ -olefin and Li—(12OH)St is assumed that,



4. The sliding mechanism according to claim 1, wherein each of the first and second members is comprised of an iron-based alloy as a base material.

5. The sliding mechanism according to claim 1, wherein the amount of the thickening agent contained in the grease 5 composition is 20 mass %.

\* \* \* \* \*